

June 30, 1931.

S. P. MILLER

1,811,953

FUEL COMPOSITION AND METHOD OF PREPARING THE SAME

Filed July 16, 1927



## UNITED STATES PATENT OFFICE

STUART PARMELEE MILLER, OF GLEN RIDGE, NEW JERSEY, ASSIGNOR TO THE BARRETT COMPANY, OF NEW YORK, N. Y., A CORPORATION OF NEW JERSEY

## FUEL COMPOSITION AND METHOD OF PREPARING THE SAME

Application filed July 16, 1927. Serial No. 206,369.

This invention relates to a new fuel composition and to an improved method of producing it.

The new fuel composition of the present invention is made up of coke oven tar freed from all or from a considerable part of the tar acids normally contained in such tar and otherwise containing tar constituents normal to coke oven tar. In particular, the new fuel composition is substantially free from decomposition products produced by distilling tar in ordinary stills with resulting decomposition of some of the tar constituents and resulting increase in pitch and carbon content.

The improved method of producing the new fuel composition includes the production of tar acids as one of the valuable products of the process.

20 Ordinary coal tar from by-product coke oven plants contains tar acids in substantial amounts. These tar acids cannot, however, be directly separated from the tar. In order to effect their separation, the tar is subjected to distillation in tar stills and the distillate oil is then subjected to treatment for the extraction of tar acids therefrom. Such distillation of the tar is accompanied by substantial decomposition of oil constituents, 25 including constituents which would otherwise be contained in the tar acid oil. If the distillation of the tar is carried to a sufficiently high temperature to secure higher tar acids or phenols, the decomposition is increased. Such increase in decomposition is 30 accompanied by increase in carbon content of the pitch residue resulting from the distillation.

The present invention provides an improved process whereby a fuel composition free or relatively free from tar acids is directly produced without the aid of distillation, and with the avoidance of decomposition resulting therefrom, and with the production of a fuel tar free from all or from a considerable part of the tar acids normally contained therein, but otherwise containing undecomposed constituents normally present in the coke oven tar.

50 According to the present invention, the hot

coke oven gases as they come from the coke ovens are cooled to a regulated temperature which is still sufficiently high to maintain the greater part or all of the tar acids in the form of vapors, and the gases are treated at such temperature with an electrical precipitator or with other means for separating therefrom the heavier tar and pitch constituents, while leaving the tar acid oils in the form of vapors. Such treatment of the gases separates therefrom a pitch product which is employed as one of the components of the new fuel composition, and which is free from increased carbon content due to subsequent distillation. The hot gases after 55 cleaning to separate heavier tar and pitch constituents therefrom are then cooled to separate clean tar acid oils, either as a single fraction or a plurality or fractions. These clean oils, being free from heavier tar and pitch constituents, can be directly extracted, for example, with caustic soda solution, to separate tar acids, therefrom, leaving a neutral oil. Naphthalene can also, if desired, be 60 separated from such oil. The neutral oil so produced is returned and admixed with the directly recovered pitch residue to form the new composite fuel composition, which will be made up of the separated pitch constituents and of the neutral oil. Both of these 65 component products are directly recovered products, which have not been subjected to further distillation, and which are accordingly free from decomposition products produced by such further distillation. The new 70 composition is also free, or relatively free, from tar acids which form another valuable 75 product of the process.

In the carrying out of the process, the hot coke oven gases, which leave the coke ovens at a high temperature, around 600 to 700° C., or higher, are cooled to a limited extent, for example, by ammonia liquor sprayed therein in the ordinary collector main, or by ammonia liquor and tar. The cooling of the 80 gases is regulated so that the tar acid oils are largely or completely retained in the vapor stated. The cooling of the gases with ammonia liquor, or with ammonia liquor and tar, in the ordinary collector main, will, due 85 90 95 100

to local cooling in contact with the ammonia liquor, result in throwing down a heavy tar which may contain a small amount of the tar acids. Most of the tar acids will, however, be retained in the gases as vapors. This heavy tar may advantageously be blended with the pitch and neutral oil as part of the new fuel composition.

The temperature to which the hot coke oven gases are cooled can be varied, even at temperatures as low as 100° C. or somewhat lower, there will still remain in vapor form a considerable amount of the lighter carbolic oils containing phenols therein. In order, however, to obtain an increased yield of tar acids, the gases should be kept at a higher temperature, for example, around 125° C. or 150° C. by regulated cooling thereof.

The hot coke oven gases, after regulated cooling thereof, are subjected to a cleaning treatment for the separation of the entrained tar and pitch constituents therefrom. This cleaning treatment is advantageously a treatment in an electrical precipitator, which will remove from the gases suspended solid and liquid particles, while leaving the vapors in the gases passing from the precipitator. Instead of using an electrical precipitator, a hot pitch scrubber can be employed, employing pitch of a composition and temperature corresponding to that carried in suspension in the gases. By a sufficiently intimate contact of the scrubbing pitch with the gases, substantially all of the suspended pitch particles can be separated therefrom, leaving a clean gas freed from suspended pitch constituents and still containing tar acid oils in vapor form.

Such treatment of the gases will result in the separation therefrom of pitch, which will be free or relatively free from tar acids, and which will differ from ordinary pitch produced by the distillation of tar in ordinary tar stills. It will be free from decomposition products produced by such distillation, and it will have a low carbon content. This directly recovered pitch product, low in carbon and free from such decomposition products, is employed in the new fuel composition of the present invention.

The cleaned gases, after separation of suspended pitch therefrom, are subjected to further cooling to separate tar acid oils therefrom. If, for example, the gases are cleaned at a temperature of 150° C. and subsequently subjected to cooling, there will be separated an oil containing constituents boiling over a considerable range of temperature and containing both the higher and the lower tar acids. If the gases are subjected to cleaning at a lower temperature, they may contain less of the higher boiling tar acids, but will still contain the greater part of the tar acid content of the coke oven gases, and particularly the lighter tar acids, such as are contained

in the carbolic oils. The cooling of the cleaned gases may take place in a single operation to a relatively low temperature, for example, around 25° or 35° C., in which case the carbolic oils will be included with the other tar acid oils in a single composite oil. By carrying out the cooling in stages, a heavier and a lighter tar acid oil can be obtained, containing respectively higher and lower boiling tar acids. The gases after the separation of the tar acid oil can then be passed to an ammonia saturator or scrubber for the absorption and recovery of ammonia therefrom; and the gases can thereafter be subjected to scrubbing for the recovery of benzol and other light oils.

The extraction of the tar acids from the tar acid oils can be effected in apparatus of the kind commonly used for extracting tar acids from distillate oils, using an aqueous solution of caustic soda or other phenol-absorbing reagent, and bringing about intimate contact of the oil with the caustic alkali solution to cause combination of the phenols or tar acids with the caustic alkali. A solution containing ten percent of caustic soda can be employed for such tar acid extraction, although a more dilute or a more concentrated solution, for example, a solution of from 25 to 35 percent strength can be employed.

The solution of tar acids in the caustic alkali can then be treated for the separation of the tar acids, for example, by treating with carbon dioxide to set free the phenols and to form a solution containing sodium carbonate; and the completion of the process can be effected by adding a small amount of sulphuric acid to the crude tar acids after separation from the sodium carbonate solution. Before the tar acids are set free from the carbolate solution, the solution may be subjected to distillation to remove other volatile constituents therefrom, such as pyridine bases, naphthalene and other dissolved oils. The tar acids separated from the carbolate solution may be subjected to further distillation and refining to give commercial tar acid products.

The oil remaining after the extraction of the tar acids will be substantially free of tar acids. It may be rich in naphthalene, in which case the extraction of the tar acids should be at a sufficiently high temperature to maintain the naphthalene in a liquid state. The extracted oil containing the naphthalene may be subjected to a cooling or chilling operation to separate part of the naphthalene therefrom, which may thus constitute a product of the process in a relatively pure form.

The extracted oil, either with or without separation of naphthalene therefrom, is employed for blending with the directly recovered pitch, or with both the pitch and

heavy tar from the collector main, to form the new fuel composition, which will thus be made up entirely of directly recovered products and which will also be free, or substantially so, from tar acids.

Where the clean oils are fractionally condensed and separately extracted for the separation of tar acids therefrom, a part only of the extracted oil may be returned for blending with the pitch to form the new fuel composition; and the remainder of the extracted oil can be employed for other purposes. The heavier oil fraction may, for example, be valuable as a creosoting material, or as an ingredient of creosoting composition, in which case only the neutral oil from the lighter oil fraction can be returned for mixture with the directly recovered pitch.

The new composite product thus produced will accordingly be made up in part of directly recovered pitch, directly recovered from hot coke oven gases, and in part of neutral oil, also directly recovered from such gases after the separation of pitch therefrom, and after the extraction of tar acids from the separated oils, and it may also be made up in part of the heavy tar from the collector main. The new composition will be free from increased carbon content due to further distillation in ordinary tar stills and in particular will be low in carbon, so that it can advantageously be stored and used without danger of separation of carbon therefrom, either in the storage tanks or in the pipe lines leading to the fuel burners.

The blending of the directly recovered pitch with the neutral oil can be carried out in an ordinary tank with suitable agitation to insure uniformity of intermixture; or the neutral oil and the directly recovered pitch can be run together into a mixing receptacle continuously, to bring about continuous blending or intermixture. If the directly recovered pitch is mixed hot with the neutral oil, it will tend to distill the lighter constituents from these oils, in which case the mixing chamber can be provided with a refluxing device to condense and return any oils so distilled. The directly recovered pitch readily blends with the directly recovered neutral oil to form a uniform fuel composition.

The invention will be further described in connection with the accompanying drawing showing in a more or less diagrammatic manner a suitable apparatus for the carrying out of the process of the invention and the production of the new fuel composition, but it will be understood that the invention is illustrated thereby and not limited thereto.

In the drawing, the coke oven block 5 has the usual uptake pipes 6 leading from the individual ovens to the collector main 7. The gases pass from the collector main through the center box 8 into the short main 9, which leads to the electrical precipitator 10. In

the goose-necks and in the collector main the hot gases are sprayed through sprays 11 and 12 with ammonia liquor or ammonia and tar supplied from a suitable source through the pipe 13. The temperature of the gases leaving the collector main is controlled by regulating the amount of spraying. Cooling of the gases causes heavy tar to be thrown out in the collector main which, together with the ammonia liquor from the sprays, collects in the center box and is drawn off into the decanter 14 from which the ammonia liquor is collected in the receiver 15 and tar is drawn off into the tank 16.

The precipitator 10 is of any suitable design. The drawing indicates a precipitator of the type shown in the copending application of G. McCloskey, Serial No. 167,338, which is especially designed for use with hot gases. The cooling is so regulated as described above that the gases passing through the precipitator will have a temperature of, for example, 125° C. or 150° C. In case a scrubber is employed for cleaning the gases, the scrubbing medium may be pitch of a temperature and composition corresponding to that of the particles removed from the gases during the cleaning operation, and with sufficiently intimate and thorough scrubbing to remove pitch particles from the gases and leave clean gases from which clean oils can be directly recovered by cooling.

The pitch thrown down in the precipitator is drawn off into the pitch receptacle 17.

The hot gases leaving the precipitator pass to condensing means which in the drawing are represented by the two condensers 19 and 20. These condensers may be of the usual type used in by-product recovery apparatus such as indirect condensers in which water is used as the cooling medium, without introducing it into direct contact with the gases. The fraction thrown down in the first condenser is drawn off into the storage tank 21 and by proper regulation of the cooling is of a nature suitable for use in creosoting compositions. The lighter fraction thrown down in the condenser 20 is drawn off into the decanter 22 from which ammonia liquid is decanted into the receiver 23 and carbolic oils are drawn off into 24. From the condenser 20 the gases pass to the exhauster 40 and to an ammonia absorber and light oil scrubber (not shown). Both the heavy oil collected in 21 and the lighter oil collected in 22 can be extracted to recover tar acids therefrom, and the neutral oils then blended with the pitch, or only the lighter oil, rich in tar acids, can be so extracted and used, leaving the heavier oil for use, e. g., as a creosote oil.

In the drawing, the tar acid extraction equipment is shown arranged for extracting only the lighter oil, although it can be similarly employed when the total clean oil is to be extracted. The oils from 24 are de-

livered to the extraction apparatus 25 by means of pump 27 through pipe 26, and are mixed with caustic soda supplied through pipe 28. The extraction apparatus may be of any suitable type such as a cylindrical tank 5 preferably with a conical bottom equipped with an agitator 29. After thoroughly mixing the caustic soda with the light oils, the mixture is allowed to settle and the solution of carbolates is separated from the extracted 10 oils and collected in the storage tank 30 while the extracted oils are drawn off into the tank 31.

The extracted oils recovered in the tank 31 15 are valuable for blending with pitch and tar to form fuel compositions. By using pitch and tar which are low in free carbon a fuel composition may be prepared from which carbon, etc., will not settle out in appreciable 20 amounts. The extracted oils are blended with the heavier products in the tank 32 to which they are supplied through the pipe 33 by pump 34. The pitch may be supplied through pipe 35 by pump 36. If hot pitch is 25 used, the two ingredients will readily blend to give a uniform mixture. When hot pitch is used, light constituents from the extracted 30 oils may be volatilized, in which case it is well to equip the mixing tank with a condenser such as is shown at 37, the condensate from which may be returned to the mixing tank. The mixing tank has an outlet 39 for 35 the fuel mixture. The mixing tank may be provided with an agitator (not shown) for promoting the blending of the pitch and extracted oil.

In addition to pitch from the precipitator, tar from the collector main may be supplied to the mixing tank through the pipe 38 in 40 suitable proportions.

The arrangement of apparatus illustrated for extracting tar acids from the light oil is 45 equally applicable for the extraction of tar acids from the creosote oil or from the total clean oil condensed from the gases, where all of the oils are condensed together and are to be extracted for the recovery of tar acids therefrom and the production of an extracted oil, which is to be blended back with the pitch 50 residue.

The apparatus illustrated provides also for the treatment of only the lighter oils rich in tar acids to recover tar acids therefrom, and to give a light extracted oil for blending with 55 the pitch residue, while giving heavier oils valuable for use directly for creosoting purposes, where they are not desired as part of the fuel composition. The blending of the light extracted oils with the pitch gives a fluid 60 fuel composition, and one readily ignited because of the contents of light extracted oils.

Where the entire clean oil recovered from 65 the gases is extracted to remove tar acids therefrom and the extracted oil is blended back with the pitch residue and with the

heavy tar from the collector main, the new fuel composition will contain practically all of the constituents normal to ordinary coal tar except the tar acids removed therefrom. Where naphthalene, as well as tar acids, is 70 removed, the fuel composition will similarly be freed from part or all of its naphthalene content. Where part of the directly recovered oil is employed as a creosote oil, the new composition will contain the remaining 75 normal constituents of the tar except for the creosote oil and the tar acids or tar acids and naphthalene, extracted or separated from the oil which is blended with the pitch and heavy tar. 80

I claim:

1. A new fuel composition comprising pitch and neutral oil constituents normally contained in coal tar in a substantially undecomposed condition, said composition being 85 free from the greater part of the tar acid constituents normally contained in the tar but containing neutral oils having boiling points corresponding to those of the tar acids, and said composition being substantially free 90 from decomposition products of the normal tar constituents.

2. The method of producing a fuel composition from hot coke oven gases, which comprises subjecting the gases to a regulated 95 cooling to condense pitch constituents therefrom while leaving tar acid oils in the form of vapors, subjecting the gases to a cleaning treatment to separate suspended pitch particles therefrom at a temperature such 100 that tar acid oils will be kept in the form of vapors, cooling the cleaned gases to separate tar acid oil therefrom, extracting tar acids from such oil, and blending the resulting neutral oil with the pitch directly separated from the hot coke oven gases. 105

3. The method of producing a fuel composition from hot coke oven gases which comprises subjecting the gases to a regulated cooling to separate pitch constituents therefrom at a sufficiently high temperature to leave creosote oil and tar acid oil in the form of vapor, passing the gases into an electrical precipitator and subjecting them therein to an electrical discharge to separate suspended 110 pitch particles therefrom, cooling the resulting cleaned gases to separate therefrom first a creosote oil and thereafter a tar acid oil, extracting tar acids from the tar acid oil and blending the resulting neutral oil with pitch directly separated from the hot coke oven gases. 115

4. The method of producing a fuel composition which comprises subjecting hot coke oven gases to cooling with ammonia liquor to 120 separate a heavy tar therefrom while leaving the gases at a sufficiently high temperature to carry tar acid oils in the form of vapors, cleaning the resulting gases by passing the resulting gases into an electrical precipi- 125 130

tator and subjecting them to an electrical discharge therein to separate pitch therefrom and to leave clean gases containing tar acid oil vapors, cooling the gases to separate tar acid oil therefrom, extracting tar acids from such oil, and blending the resulting neutral oil with the pitch and tar directly recovered from the coke oven gases.

In testimony whereof I affix my signature.  
**10 STUART PARMELEE MILLER.**

**15**

**20**

**25**

**30**

**35**

**40**

**45**

**50**

**55**

**60**

**65**